

# UNITED STATES PATENT OFFICE.

ROBERT TRIPMACHER, OF SCHWEIDNITZ, GERMANY.

## PROCESS RELATING TO REFRACATORY SUBSTANCES.

No. 930,575.

Specification of Letters Patent.

Patented Aug. 10, 1909.

Application filed April 28, 1909. Serial No. 492,671.

To all whom it may concern:

Be it known that I, ROBERT TRIPMACHER, a subject of the German Emperor, and residing at Schweidnitz, Silesia, German Empire, have invented certain new and useful Improvements in Processes Relating to Refractory Substances, of which the following is a specification.

It is well known that certain minerals, especially those belonging to the spinel group, both natural and artificial, are refractory in a high degree. One of these minerals which withstands particularly high temperatures is, for instance, chrome-iron ore (chromite), whose chemical formula is  $\text{FeCrO}_4$ . This material has consequently long been employed in pieces for lining the sole of the hearth of many kinds of metallurgical furnaces and the like.

23 The reason why chrome-iron ore is not generally employed for other than the above-mentioned purpose is the difficulty experienced in uniting or binding the particles of the pulverized mineral. For in practice it is necessary that the degree of cohesion should be sufficient to enable the material to withstand the pressing or other treatment in making blocks, bricks, or like shaped pieces, as also all the phases of the firing or baking process; and when once given a firm, solid form it must be capable of retaining such for a sufficient period of time in industrial use.

Prior methods of overcoming the difficulty, such as the employment of artificial (i.e. chemically manufactured) aluminium hydrate ( $\text{Al}_2(\text{OH})_6$ ) as binding medium for the pulverized chrome-iron ore, have not proved satisfactory viewed from an economical standpoint; or the agents which it has 43 proposed to add to the disintegrated chrome-iron ore for the purpose of binding it have been found unpractical, since owing to their nature and the percentage in which they have to be added they too greatly diminish the degree of refractoriness which constitutes the most valuable feature of the ore.

According to my invention I employ as binding-agent for the pulverized chrome-iron ore materials which are for the most part removed again in the course of the treatment, and yet insure thorough cohesion in all stages of manufacture, and yield a final product which has lost little or nothing of the highly refractory character of the ore.

55 In making my new binding-agent I dissolve in molasses or a similar saccharine so-

lution boric acid or a borate (e.g. borax), together with a small quantity of chromic acid or a chromate (e.g. potassium or sodium chromate, or potassium or sodium bichromate), and very finely emulsify naphtha or an equivalent substance in this liquid. Or where expense is a matter of less importance boric acid or borate may be dispensed with, a correspondingly greater quantity of chromic acid or chromate being then used. I have also found it advantageous to add to the mass small quantities of cryolite or other suitable fluorid such as fluor-spar, for the purpose of permanently intensifying the cohesion of the highly refractory particles after evaporation of all other binding-media.

In practice I prefer first to dissolve the boric acid in hot water, to obtain a concentrated solution, as it is but difficultly soluble in cold water; to this solution I add the chromic acid; and then mingle the molasses. Hereupon I add the naphtha and thoroughly stir to insure uniform distribution. This results in the naphtha distributing itself in a state of extraordinarily fine emulsion. Apparently this is due to the percentage of alkaline constituents of the molasses. With the liquid so obtained the pulverized chrome ores can be bound, pressed in the ordinary manner, dried, and fired at a sufficiently high temperature. The product retains its coherence, in all phases of the drying and firing operations as there is always a binding constituent present.

The part played by the chromic acid is an extremely peculiar and wholly unexpected one. It will be found that the briquets or blocks formed when a binding-liquid containing chromic acid is used, stiffen after a short time (a few hours) in such manner that they can be shaped by hand without the employment of hydraulic presses. They can then be pressed at once in the ordinary manner without any danger of their falling to pieces. In fact this subsequent pressing may even be omitted, or for instance only employed when it is desired say to stamp the manufacturer's name or to render the edges of the blocks sharper. A particular advantage of this method is that blocks of other shape than the usual bricks can be readily manufactured, since the high pressure otherwise requisite is unnecessary and all danger of the blocks cracking or collapsing is avoided. Chromic acid, therefore, in

an altogether surprising manner proves to be an unusually suitable ingredient for agents for binding highly refractory material. A further advantage of the chromic acid is that on firing it is converted into chromic oxide, that is, it appears in the finished material as a product of substantially the same highly refractory character as the original material.

10 10 When a refractory material is required which will thoroughly resist the reducing flame, which is not sufficiently the case with chrome ores, there may be employed instead of these some other refractory substance 15 such as native or burnt magnesite, refractory clay, chamotte, or mixtures of these substances, bound by the new liquid.

Having thus described my invention, I declare that what I claim is—

20 1. The process of binding refractory substances, consisting in treating the same in pulverized condition with a liquid which consists of a saccharine solution, and a chromium compound, in which naphtha is emulsified, substantially as described.

25 2. The process of binding refractory substances, consisting in treating the same in pulverized condition with a liquid which

consists of a saccharine solution, and boron and a chromium compound, in which naphtha is emulsified, substantially as described. 30

3. The process of binding refractory substances, consisting in treating the same in pulverized condition with a liquid which consists of a saccharine solution, and a chromium compound, in which naphtha is emulsified, with the addition of a fluorid, substantially as described.

4. The process of binding refractory substances, consisting in treating the same in 40 pulverized condition with a liquid which consists of a saccharine solution, and chromic acid, in which naphtha is emulsified, substantially as described.

5. The process of binding refractory substances, consisting in treating the same in 45 pulverized condition with a liquid which consists of a saccharine solution, and boric and chromic acid, in which naphtha is emulsified, substantially as described.

In testimony whereof I affix my signature in presence of two witnesses.

ROBERT TRIPMACHER

Witnesses:

SIEGFRIED LUSTIG,  
ERNST KATZ.